

## [54] STRIPPING OF DIFFUSION TREATED METALS

[75] Inventor: Alfonso L. Baldi, Wynnewood, Pa.

[73] Assignee: Alloy Surfaces Company, Inc.,  
Wilmington, Del.

[21] Appl. No.: 147,191

[22] Filed: May 6, 1980

## Related U.S. Application Data

[63] Continuation-in-part of Ser. No. 98,654, Nov. 29, 1979,  
Pat. No. 4,290,391, Ser. No. 25,456, Mar. 20, 1979, and  
a continuation-in-part of Ser. No. 963,313, Nov. 24,  
1978, abandoned, Ser. No. 851,504, Nov. 14, 1977, and  
Ser. No. 752,844, Dec. 21, 1976, Pat. No. 4,208,453.[51] Int. Cl.<sup>3</sup> ..... C23F 1/00[52] U.S. Cl. ..... 427/253; 134/3;  
156/664; 156/665[58] Field of Search ..... 134/3, 2; 427/252, 253;  
156/665, 664

## [56] References Cited

## U.S. PATENT DOCUMENTS

3,458,353 7/1969 Baldi ..... 156/665  
3,622,391 11/1971 Baldi ..... 156/665  
3,833,414 9/1974 Grisik et al. ..... 134/3

4,032,359 6/1977 Fisher et al. ..... 134/3

Primary Examiner—Ralph S. Kendall  
Attorney, Agent, or Firm—Connolly and Hutz

## [57] ABSTRACT

Chromized nickel- and cobalt-based superalloys have alphachrome phase formed during chromizing, and the amount of that phase is diminished by one or more treatments with alkali-permanganate solution and intervening removal of permanganate reaction product film as by acid dip. A kit of such solutions can be prepared. Low-alloy steel steam boiler tubing can have chromized interior and aluminized exterior, and long lengths chromized without a perfectly sealed retort around it can have end caps fitted with extra pack to reduce oxygen penetration to interior. Chain saw cutter blades can be chromized and carburized. Stripping of aluminized coatings from superalloys with fluoride-containing nitric acid solution is improved by follow-up treatment with fluoride-free nitric acid solution. Smut that forms on ferrous surface during cleaning is chemically removed by first depositing a nickel flash plating on smut-containing surface, and then dissolving the nickel plating by treatment with aqueous nitric acid containing a little halide ion.

3 Claims, 2 Drawing Figures



*Fig. 1.**Fig. 2.*

## STRIPPING OF DIFFUSION TREATED METALS

The present application is in part a continuation of applications Ser. No. 98,654 filed Nov. 29, 1979 (U.S. Pat. No. 4,290,391 granted Sept. 22, 1981), Ser. No. 25,456 filed March 30, 1979, and a CIP Ser. No. 963,313 filed Nov. 24, 1978, (subsequently abandoned), Ser. No. 851,504, filed Nov. 14, 1977, and Ser. No. 752,844, filed Dec. 21, 1976, (U.S. Pat. No. 4,208,453 granted June 17, 1980). The entire contents of Ser. Nos. 752,855, 963,313, and 25,456 are incorporated herein as though fully set forth and some of those contents are copied over herein.

The present invention relates to the treatment of metals to improve their usefulness.

Among the objects of the present invention is the provision of novel coating techniques as well as novel treating compositions and treated products, that have desirable properties.

Additional objects of the present invention include compositions and techniques for confining protective diffusion coatings to desired locations on workpieces such as jet engine components to be protected by the coatings.

The foregoing as well as further objects of the present invention will be more fully understood from the following description of several of its exemplifications, reference being made to the accompanying drawings wherein:

FIG. 1 is a somewhat diagrammatic illustration of a set-up for diffusion coating pursuant to the present invention; and

FIG. 2 is a longitudinal sectional view of one end of tubing prepared for a diffusion coating illustrative of the present invention.

According to one aspect of the present invention nickel-based and cobalt-based superalloys are very easily chromatized to form heavily chromized cases that are then made exceptionally free of alphachrome phase. Because of the desirability of cases containing a high chromium content for improving the resistance of such superalloys to corrosion particularly by sulfur-containing atmospheres, several processes have been developed for chromizing these metals. Some of these prior processes are disclosed in the parent applications, and one such process is the gas-phase diffusion coating by heating the superalloy workpiece while it is suspended in a retort the floor of which is covered with a mixture of finely divided chromium particles, inert diluent such as powdered alumina, and an activator such as ammonium chloride.

When it is attempted to provide maximum concentrations of chromium in a diffusion case, some alphachrome phase seems to form no matter what technique is tried to prevent it. The presence of such phase is recognized as undesirable because it imparts excessive brittleness to the diffusion case.

Pursuant to the present invention the chromizing is carried out to the extent that alphachrome is formed, and then the alphachrome is removed by treatment with an aqueous solution of alkali metal permanganate and alkali metal hydroxide. This treatment leaves a dark-colored reaction product which is believed to contain little or none of the removed chromium. The alkaline permanganate solution should be a temperature of at least about 100° F. to effect alphachrome removal in reasonable periods of time, and the hotter the solution

the more rapid and complete is its action. One exemplification of such a process is:

## EXAMPLE 1

A cylindrical diffusion coating retort 10 as in FIG. 1, made of plain carbon steel, has its floor 12 covered to a depth of about 1½ inches with a layer 14 composed of, by weight:

20 parts chromium powder 10 to 20 microns in size  
10 80 parts tabular alumina granules 100 to 200 microns in size  
10 ¾ NH<sub>4</sub>Cl powder

These ingredients are mixed together so as to make a layer of fairly uniform composition, and does not have to be pre-fired.

On layer 14 is placed a multiplicity of retaining tubes 20 also of plain carbon steel, each holding B-1900 superalloy jet engine blade 30 the airfoil portion 32 of which is embedded in a diffusion coating pack 22. Pack 22 is composed of, by weight:

25 45 parts chromium powder 10 to 20 microns in size  
23.5 parts nickel powder 10 to 50 microns in size  
3.6 parts aluminum powder 20 to 100 microns in size  
27.9 parts fine alumina powder that passes a 325 mesh screen

25 0.5 part NH<sub>4</sub>Cl powder

This mixture is pre-fired by heating for 10 hours in a plain carbon steel retort at 1900° F. in a hydrogen-bathed atmosphere without a workpiece, the pre-fired 30 pack then crushed to pass a 200 mesh screen and 0.5 part NH<sub>4</sub>Cl powder is added to it to make up for the NH<sub>4</sub>Cl driven off by the pre-firing.

To avoid depleting some of the chromium from the pack 22 when it is subjected to the pre-firing, the pre-firing retort can be previously chromized, or can be a high-chromium alloy such as Inconel 600.

For loading tubes 20, the individual blades 30 are first held by fitting their roots 34 in apertures in a supporting table, these apertures being too small to receive blade 40 flange 36. The airfoils 32 are thus pointed upward and a tube 20 is placed over each of them. The pre-prepared pack 22 is then poured into the tube and tamped in place so that it stays there and does not pour when the tube is inverted. The tube should have only a small clearance, 45 about ½ centimeter or less, with respect to the blade flange 36 and support, to keep pack 22 from pouring out the bottom of the tube during the loading and tamping.

The tubes so loaded are then inverted and placed over layer 14 in retort 10, a gas supply tube 38 and 50 thermocouple 40 inserted in the retort with the gas supply tube immersed in powder layer 14, the retort covered by a loosely fitting cover 16 or by placing another retort over its open top, and the assembly subjected to a diffusion coating heat in an outer retort through which hydrogen is passed as described in U.S. Pat. No. 3,764,371, while argon at a slow rate, about 5 standard cubic feet per hour, is fed into retort 12 through tube 38 which has many perforations 39. The assembly is brought to 1925° F. and maintained within 60 plus or minus 25 degrees of that temperature for 16 hours, after which it is permitted to cool.

The loaded tubes are removed from the cooled retort and the blades 30 removed from pack 22 after that pack is loosened as by jarring the tube. The roots 34 of the blades now show a case about 0.7 mil thick containing a maximum of about 35% chromium and a very small amount of alphachrome phase. The airfoils 32 on the other hand have a case with two chromium diffused

zones. The outer zone is a little over 1 mil thick containing a maximum of about 75% chromium and is essentially alphachrome. The inner zone is essentially gamma nickel containing a maximum of about 35% chromium.

The alphachrome phase is removed from the blade roots by now dipping the roots for about 10 minutes in a 180° F. solution in water of 5%  $\text{KMnO}_4$  and 5%  $\text{NaOH}$ , then rinsing and dipping them for a few seconds in 10%  $\text{HCl}$  in water to remove the film formed by the alkaline permanganate, and the alkaline permanganate dip repeated. The roots now show no alphachrome phase. The entire blade can be so treated, if desired, inasmuch as this treatment has a negligible effect on the heavy alphachrome phase on the airfoils.

The blades are then aluminized by subjecting them to an aluminum diffusion pack treatment at  $1925^\circ \pm 25^\circ$  F. for 12 hours in the manner described in U.S. Pat. No. 4,041,196, the roots being kept imbedded in a masking pack in order to keep them from being aluminized. The aluminizing increases the case depth over the airfoil to close to 3 mils maximum, brings up the aluminum content of the case to over about 25%, and breaks up the alphachrome phase into a multiplicity of small islands. As described in U.S. Pat. No. 4,041,196 such a case does not have the undesirable unduly brittle character of a continuous alphachrome phase, and because of its high chromium content is particularly resistant to sulfidation attack. The aluminizing also makes it highly resistant to oxidative attack.

Repeating the chromizing on fresh blades can give a chromized airfoil case with an outer high-chromium-content zone a little over 0.5 mil thick, the blade roots then having their alphachrome content readily removed by a 5 minute dip in the 5%  $\text{KMnO}_4$ —5%  $\text{NaOH}$  solution at 160° F., followed by a few seconds dip in 18%  $\text{HCl}$  in water.

The cooling down from the aluminizing step can be effected at a rate rapid enough to subject the vane to the first step of a heat treatment usually followed by an ageing step to give nickel-base superalloys their maximum strength as described in U.S. Pat. No. 3,824,122.

The chromizing treatment can if desired also be effected with masking of a blade root or vane buttress, using any of the procedures described in Ser. No. 752,855 or U.S. Pat. Nos. 3,801,357 and 3,785,854. When masking a surface on a nickel-base superalloy, care should be taken to limit the amount of nickel powder located close to the surface being masked. The large amount of such powder specified in Example 1 of Ser. No. 752,855 can cause inter-granular attack of the nickel-base substrate if the "first layer" specified in that example, is omitted. Ser. No. 752,855 does indicate elsewhere that such omission can be made but if made the nickel powder should be reduced to about 1/5 the amount shown in that Example 1.

To avoid the foregoing inter-granular attack problem completely, masking of nickel-base superalloys can be performed without any nickel powder as by using either the masking powder pack or slurry technique of U.S. Pat. No. 3,801,357. Such a slurry can also have the binder and solvent of Ser. No. 752,855.

The alkaline permanganate treatment is best applied before the aluminizing step, and can be effected at temperatures as high as the boiling point of the treating solution, in which case a single dip is sometimes adequate to remove all alphachrome if only present in small amounts. This treatment can also be conducted at temperatures as low as about 100° F. where a multiplicity of

dips is generally needed. At 150° F., two dips are adequate, but three dips are best used when the alkaline permanganate solution is at 130° F.

The acid treatment between the alkaline permanganate dips can be with inhibited or uninhibited acid, preferably the former if the acid treatment is prolonged for more than a few seconds. It can be completely omitted in which event the alkaline permanganate treatments at temperatures of 200° F. or below are extended to  $\frac{1}{2}$  hour or longer. Other strong mineral acids like  $\text{H}_2\text{SO}_4$ ,  $\text{H}_3\text{PO}_4$ ,  $\text{HNO}_3$  and  $\text{HBr}$  can be used, and the acid concentration is preferably about 5 to 15% by weight. Without an acid after-treatment a film of adherent dark-colored reaction product left on the workpieces by the alkaline permanganate treatment can be removed by other techniques such as sand blasting.

The alkaline permanganate solution can be prepared with any alkali metal hydroxide and should have a pH of at least about 13, although alkalinites as low as 11 can be used by prolonging the dips and/or repeating them more times. The concentration of the permanganate should also be above about 0.1%, but below about 3% strength the dip times need to be lengthened.

Increasing the concentration of the permanganate and/or the alkali, speeds the action somewhat. Like the alkali, the permanganate can be of any alkali metal. The action of the alkali-permanganate bath seems to be that of oxidizing chromium in the alphachrome form, and its effect extends to depths of as much as  $\frac{1}{2}$  mil into the case. This is the zone in which alphachrome usually forms.

It is helpful to provide, for the alphachrome removal, a kit made up of a solution of alkali combined with permanganate, and a separate solution of a mineral acid, preferably inhibited hydrochloric acid. Such a kit can be a convenient article of commerce, containing the separate solutions separately bottled in unbreakable plastic bottles. Inasmuch as the volume of each solution determines the amount of material that can be immersed in it, both solutions can have about the same volume. However the mineral acid is available in concentrations that require dilution, whereas the alkali-permanganate solution is conveniently used at a concentration near its maximum, so that to reduce costs the kit can have the acid at a concentration that requires dilution to two or three times its volume before use.

For maximum cost-effectiveness the quantity of permanganate and/or acid can be adjusted so that both solutions become exhausted at about the same time. The rate of permanganate exhaustion is subject to considerable more variation than that of the acid exhaustion, but in general the total weight of permanganate ion can be about one to two times the total weight of anhydrous acid, in the acid solution.

It is also practical to have the alkali and/or the permanganate of the kit in dry or undissolved condition inasmuch as this reduces the total weight and bulk of the kit. The proportion of these two ingredients can then be from about 30:70 to 70:30 by weight. The mineral acid of the kit can be replaced by inhibitor such as rosin amine acetate. Such inhibitor can be present dry or dissolved in a little water, so that it can be mixed with uninhibited acid such as hydrochloric acid, by the user. The amount of inhibitor is generally about 0.1% to about 1% by weight of anhydrous acid.

The alphachrome removal of the present invention can be used to reduce or eliminate the alphachrome content of the airfoil portion of the blades produced in

Example 1, but because the alphachrome content of the airfoils is much greater than that of the roots, the alkaline permanganate treatment takes several times as long, even when conducted in stages. In general it is preferred to remove no more than about 5 milligrams of chromium per square centimeter of surface by this treatment.

Other jet engine turbine parts such as vanes can also be given the treatment of Example 1. Such vanes have buttresses, which like the roots of blades, are mounting portions preferably free of alphachrome while their airfoils are improved by an aluminized alphachrome that leaves the alphachrome in separated islands.

The coating technique of Example 1 is particularly desirable and when used to form chromized cases by a gas-phase chromizing as there shown for the blade roots, provides such cases with a minimum of alphachrome phase. Where such case is formed with a maximum chromium content of about 30% or less, no alphachrome phase at all can generally be detected and no alphachrome removal step is needed. Combining the gas-phase coating with the pack coating as in Example 1, makes it unnecessary to provide separate supports for holding the workpieces exposed to the gas-phase.

In general the chromizing mixture 14 for the gas-phase coating can have as little as 2% and as much as 80% chromium, preferably 5 to 80%, and other inert diluents like fired kaolin can be used in addition to or in place of the alumina. The heavy chromizing pack 22 should have at least about 2% aluminum to minimize the formation of oxide inclusions, but its nickel content can be reduced to about the same level as the aluminum content. Its chromium content should be at least about 40%, preferably at least 60%, of the total of all its metallic ingredients, and the aluminum content should be not more than one-fifth, preferably not more than one-ninth, the chromium content. Other activators such as ammonium bromide, elemental iodine and ammonium bifluoride can be used.

There should be sufficient inert diluent, for instance at least about 25% by weight, in the pack 22 as well as in mixture 14, to keep the metal particles in them from sintering together or to the workpiece, tube or retort. It is also helpful to have pack 22 of such non-fluent nature that the packed tubes 20 can be placed on and removed from mixture 14 without having any material amount of that pack fall into that mixture and thus contaminate it. By avoiding such contamination, both the pack 22 and the mixture 14 can be reused. Mixture 14 can be made more fluent as by using a fluent form of alumina for its inert ingredient. Tabular alumina powder having particles about 100 to 300 microns in size are suitable for this purpose.

The retort 10 and tubes 20 become fairly heavily chromized after a few runs, so that there is no need to make them of anything more expensive than inexpensive stainless steel.

The process of Example 1 can be used with other nickel-base superalloys such as U-500, IN-738, IN-713 or U-700, as well as with cobalt-base superalloys including WI-52, Mar-M 509, PWA 657 and X-40, to prepare a chromized, or a chromized then aluminized, product. If desired the chromizing can be uniformly applied over the entire workpiece either by the gas phase arrangement omitting pack 22, or by pack diffusion in which event the entire workpiece is imbedded in the pack with or without the help of tubes 20. The gas phase treatment applies less chromium as well as very little or no alpha-

chrome, and does not increase the workpiece dimensions very much. When it applies a chromized case about 0.7 mil thick, about one-third that case thickness is thickness that adds to the original workpiece dimension. The remainder of the case thickness represents the original surface of the workpiece.

The alphachrome-removal treatment described above can be effected on chromizing cases regardless of how those cases are produced. It extracts alphachrome 10 chromium, but does not appear to attack other phases in the chromized case, so that the total chromium loss caused by this treatment is very small.

Hollow engine vanes or other types of hollow workpieces can also be diffusion coated in accordance with 15 Example 1, and if the hollow interior opens on its exterior, some coating will also form in that interior. Where the internal surface of a hollow workpiece does not require heavy case formation the hollow interior need not be packed with a diffusion-coating pack but can merely be left in communication with the gas space in the retort. To improve the gas phase chromizing of such interiors, without complicating the operation unduly the interior can be coated with a uniform layer of chromium particles as described in application Ser. No. 15 089,949 filed Oct. 31, 1979 (subsequently refiled). Alternatively, the retort can be equipped with a gas circulator such as the rotor of U.S. Pat. No. 3,353,936 to propel the retort gas through the workpiece interior during the chromizing operation. A series of hollow vanes can thus be disposed around the periphery of such rotor, each vane having the passageway to its interior located close to the rotor margin and oriented to directly receive gas propelled by the rotor.

The diffusion-coating powder mixture used with the gas phase chromizing need not cover the retort floor but can leave a portion of the floor bare to receive workpieces and/or the rotor. Indeed the diffusion-coating powder mixture can be held entirely off the floor, in baskets for example as in U.S. Pat. No. 3,353,936.

When chromizing the interiors of very long lengths of tubing in a furnace without enclosing the tubing in a gas-tight retort, there is a tendency for oxidation of the surface being chromized. This tendency can be reduced by closing the ends of the tubing with caps that contain an extra supply of chromizing pack or other material that combines with or blocks passage of oxygen and moisture. FIG. 2 shows such a modified capping arrangement.

In FIG. 2 the end of a steam boiler tube 50 having an 50 inside diameter of 2 inches and a  $\frac{1}{2}$  inch wall thickness is covered by a cap 52. The cap is a welded-together assembly of an end wall 56 and a tubular flange 58 which loosely fits over the end of pipe 50.

The tube 50 is filled with diffusion coating pack, more pack is poured into the cap 52, and the cap then fitted over the tubing end. A little extra pack 60 thus becomes located beyond the end of the tube and reduces the tendency for any oxidizing effect in the interior of the tube. If there is a little clearance 62 between the outside 60 surface of tube 50 and the inside surface of flange 58, the flange 58 can be tack-welded to the tube for the purpose of securing the cap in place. No significant clearance is needed, and the cap can then be frictionally held in place.

The internal pack is a highly fluent composition that is easily poured into place before the heat, and some of it may find its way into the clearance space 62. It is also readily removed after the heat is completed, using a

minimum of mechanican poking and the like. As described in application Ser. No. 752,855 such a pack is particularly desirable for packing of cramped recesses in the interior of workpieces, such as in the narrow bores described above, or in hollow jet engine blades, or the like.

Example 2 of application Ser. No. 752,855 describes the diffusion coating of steam generator high pressure tubing made of Croloy alloy (1.9 to 2.6% Cr, 0.97 to 1.13% Mo, 0.15% C, balance essentially iron) having a  $\frac{3}{8}$  inch bore and a  $\frac{1}{2}$  inch wall thickness. That diffusion coating included the chromizing of the tube's interior and the aluminizing of the tube's exterior. The chromized case was 1.8 to 2.3 mils thick, with an outer portion about 0.3 mil thick rich in chromium carbide, and an inner portion of columnar chromized structure. This case is particularly effective in reducing erosion of the internal tube surface by rapidly moving high pressure steam.

The aluminized outer surface prolongs the life of the tube in a coal- or oil-fired furnace where it is subjected to combustion atmospheres at temperatures as high as about 100° F.

For some steam-generating arrangements lengths of steam-generating tubes have one end bent back 180 degrees to form cane-shaped units which can have their ends welded to additional lengths to form a continuous furnace tube assembly. The packing of the bores of such "canes" for diffusion coating, and the subsequent pack removal after coating, is greatly simplified by the use of fluent packs as described in application Ser. No. 752,855.

Any ferrous base steam boiler tubing is improved by the last-mentioned diffusion coatings. Those plain carbon and low alloy steels that will form the chromium carbide stratum with the underlying columnar chromized case will show very little abrading loss when used with high pressure steam. Such abrasion by the steam causes the steam to carry along with it the abraded particles and they can damage the vanes and blades of turbines driven by the steam. For such pressurized use the boiler tubing should have a wall thickness of at least about 3/16 inch.

The external surfaces of boiler tubing are also made more resistant to corrosion as a result of the aluminizing or the chromizing described above, even the minor chromizing effected when only the interior of such a tube is packed with the diffusion chromizing mix.

It is not necessary to diffusion coat the external surfaces of such tubes or to diffusion coat those external surfaces with aluminum. The internal bores of such tubes can be chromized for instance without the use of a covering layer on their exterior. Such chromizing in the retort arrangement described in Example 2 of application Ser. No. 752,855 will produce a distinct outer chromized case in addition to the above-described internal case, but the outer case will generally not show the carbide stratum and will have less chromium pick-up.

The foregoing inner and outer coatings can be applied to tubes as long as 40 feet or more in length, whether those tubes be straight or cane-shaped. For such long tubes it is desirable to effect the diffusion coating uniformly along the tube lengths, and to this end the diffusion coating temperature along the length of the tube can be closely controlled.

As also pointed out in application Ser. No. 752,855 an argon washing atmosphere can be maintained in place of the hydrogen washing atmosphere of its Example 2,

without significantly different results. Because of its expense, the flow of argon should be reduced to a very small rate by back pressuring it equivalent to 1 to 2 inches of water. Alternatively, that diffusion can be effected in a glass-sealed retort with an autogenously generated atmosphere.

Chain saw cutter blades are examples of other workpieces that can be diffusion coated to improve their operation. In some cases the cutting edge of a chain saw blade is the narrow edge face on a steel flange, one surface of the flange being very hard and the opposite surface of the flange being relatively soft. The edge face connects those two surfaces and is preferably tapered so that the edge of the harder surface projects out further than the edge of the softer surface, thus providing good cutting action. During use the edge face wears with the softer portion wearing faster than the harder portion so that the cutting effectiveness of the edge face is maintained quite well.

More generally however the cutting edge of such a blade can be diffusion chromized throughout to greatly harden it, particularly if the blade is made of low alloy high-carbon steel. To provide maximum hardening the workpiece can be subjected to carburizing conditions as well as to chromizing, so that the chromium that diffuses into the surface of the blade forms a carbide higher in carbon content than  $\text{Cr}_{23}\text{C}_6$ .

The carburizing and chromizing can be effected in separate operations, or in a single step. The following example shows a chromizing followed by a carburizing, effected on a low alloy high-carbon steel of the following composition:

0.65% carbon  
0.3% manganese  
0.75% nickel  
0.5% chromium  
0.15% molybdenum  
balance essentially iron

#### EXAMPLE 2

These cutters are cleaned and imbedded in a pack made up of a pre-fired mixture of 20% chromium powder and 80% alumina powder, by weight, to which mixture is added  $\frac{1}{2}\%$  ammonium chloride. The pack is held in a retort which is then heated in a hydrogen-bathed atmosphere to 1600°-1650° F. where it is kept for 5 hours. Upon cooling the cutters show a chromized case 0.4 to 0.5 mil thick.

The chromized cutter blades are then carburized in a carbon monoxide atmosphere where they are held at 1550° F. for 2 hours. The resulting blades show a small increase in case depth as well as long life. Other carburizing techniques such as described in the Kirk Othmer Encyclopedia of Chemical Technology, Second Edition, Volume 13, pages 304 through 308 (1967), can also be used with equivalent results.

Both the chromizing and the carburizing can be carried out in the same retort, as for example by suspending the cutter blades in the retort, then introducing a chromizing gas such as described in U.S. Pat. No. 3,222,212, after which such gas is displaced by carbon monoxide or methane or other carburizing atmosphere. The temperature of both treatments can be close to each other, or several hundred degrees apart, as desired. Simultaneous chromizing and carburizing is not very effective.

The weight gain of the blades can be followed to make sure the above-noted high proportion of carbon-to-chromium has been introduced into them. Such pro-

portions give very long-lived cutters, but lower proportions can be used.

If desired the chromizing can be accomplished with a pack that contains a small amount, about 1 to 2% by weight, of metallic magnesium powder. This further improves the durability of the case whether or not it is subsequently carburized.

Aluminide coatings can be removed from superalloys where fresh coatings are needed, and even to vary the coating thickness, by the processes described in U.S. Pat. Nos. 3,458,353 and 3,622,391. These processes use dips in stripping solutions of aqueous nitric acid containing dissolved fluoride. A preferred stripping solution contains about 3 to about 20 weight percent of dissolved fluoride computed as hydrogen fluoride.

While such stripping solutions are highly effective at moderate temperatures, e.g. 50° to 115° F., their action on some coatings is sometimes slow. The stripping can be accelerated by a follow-up dip in essentially fluoride-free aqueous nitric acid having about 10 to about 30 weight percent acid, for at least about 5 minutes. Even speedier removal is effected by repeating the fluoride-containing and fluoride-free nitric acid dips, with an intervening water rinse.

A particularly desirable sequence is shown in the 25 following example.

### EXAMPLE 3

A number of INCO 713 aluminized first stage blades are subjected to the treatment steps:

(a) Clean with a blast of dry 220 grit aluminum oxide propelled by a jet of air from a 30 psig source.

(b) Immerse for 30 minutes at 80°-90° F. in a fluoride-containing nitric acid solution prepared by dissolving 2 ounces of ammonium bifluoride and 10 fluid ounces of 70% nitric acid, in sufficient water to make one gallon.

(c) Rinse with running water.

(d) Rinse ultrasonically in water for two minutes.

(e) Dip for 30 minutes at 90°-100° F. in aqueous nitric acid containing 17 weight percent technical grade 40 HNO<sub>3</sub>.

(f) Rinse in running water.

(g) Rinse ultrasonically in water for two minutes.

(h) Repeat the sequence of steps (b) through (g) two more times.

(i) Grit blast as in step (a).

Even better results are obtained when the fluoride-free acid solution of step (e) contains 25% HNO<sub>3</sub>. The temperature of the fluoride-free acid bath can be as low as about 60° F. and as high as about 125° F., and still 50 provide very good action. Higher temperatures tend to generate vapors that make the bath a serious health hazard, and are best avoided. For the same reason the fluoride-containing bath is best operated at from 50° to about 115° F.

The chemical attack of the acid dips stops of its own accord after the aluminide coating is entirely removed, so that there is no great danger in prolonging the dip treatments. However dips longer than about 30 minutes are not particularly helpful and unduly prolong the treatment.

The rinsing between fluoride-free acid dip and a fluoride-containing acid dip that follows, can be omitted. The rinsing between the fluoride-containing acid dip and the fluoride-free acid dip that follows, is helpful in 65 that it keeps the fluoride-free acid from accumulating too much fluoride that can be carried over from the fluoride-containing acid dip. The fluoride-free acid dip

should have less than about 0.1% and preferably less than 0.05% fluoride content.

The rinsing liquid need not be water, but can be some other liquid such as cellosolve, chloroform, methylethylketone, alcohols or mixtures of such liquids. Rinsing should be effected after the last acid treatment, before the workpieces are cleaned and dried.

According to the present invention chromizing can also be effected to provide smooth hard low-friction surfaces on hardened steel. Thus gun barrels of high-carbon steel can have their internal bores chromized to form a hard case not over 1 mil thick that improves the operation of the barrel. Barrels having a caliber of 30 hundredths of an inch, or even less, can be improved 15 this way.

It is generally awkward to make ferrous metal surfaces scrupulously clean. The awkwardness principally involves the formation of smut on the ferrous surface, particularly if it has been subjected to an electrolytic or acid treatment. The smut is probably the residue of some of the resistant constituents of the ferrous metal left behind when the surface of the metal is attacked, and the best technique for removing the smut has been mechanical brushing. Because brushes so used tend to wear out fairly rapidly, the operation of fast-moving production cleaning lines that include brushing is difficult to make completely automatic.

According to another aspect of the present invention the brushing off of the smut is replaced by the steps of 30 depositing on the smutty surface a flash coating of nickel and then subjecting the thus-coated surface to the action of aqueous nitric acid containing a little halide such as Cl<sup>-</sup>. This rapidly dissolves the nickel coating and also removes the smut. This is exemplified as follows.

### EXAMPLE 4

A coil of two mil thick SAE 1010 steel foil is passed through a series of tanks in which it is treated in the following sequence of steps each taking about 1/6 minute:

(a) Alternating current (60 Hertz) electrolytic action as a bipolar electrode at 50 amperes per square foot in an aqueous solution containing 5% NaOH and 5% sodium 45 silicate and held at 150° F.

(b) Reciprocal bipolar electrode electrolytic action at the same current density and in the same bath as in step (a).

(c) Rinse in tap water.

(d) Dip in 1% by weight aqueous inhibited hydrochloric acid.

(e) Rinse in tap water.

(f) Passage through a nickel flash plating bath in which it is cathodically treated for three minutes at a 55 current density of 20 amperes per square foot. The bath is an aqueous solution of 213 grams NiCl<sub>2</sub>.6H<sub>2</sub>O and 35 cc. 20% aqueous HCl, in 500 ml. water and is held at about 70° to 100° F.

(g) Rinse in tap water.

(h) Dip in 20% by weight aqueous nitric acid containing 0.1% by weight hydrochloric acid.

(i) Rinse in tap water.

After emerging from the final rinse the foil is clean and no smut is detectable. It can now be loosely coiled as described in U.S. Pat. No. 3,222,212 for diffusion coating, or given any other kind of coating.

The nickel flash can be deposited from acid or alkaline plating baths and need only weigh about 0.05 milli-

gram per square centimeter. Greater coating weights do not help the smut removal significantly and coating weights over about 0.3 milligram per square centimeter generally take too long to apply and are too expensive. An electroless Nickel flash can be used but it is not as effective.

The smut removal of the present invention can be effected on high-carbon steels as well as on alloy steels including stainless steels and does a very good job on flat or curved surfaces. Surfaces that are too concave or convex should be plated with the help of anodes so shaped and located that a fairly uniform flash coat is deposited, in order to make sure the flash is deposited all over the surface in the least time.

The nitric acid content of the flash-removing solution can range from about  $\frac{1}{2}\%$  to about 40% by weight, and should contain about 20 to about 200 times as much nitric acid as halide ion. While hydrogen chloride is a very convenient source of halide ion, any chloride, bromide, iodide or fluoride that dissolves and dissociates in the nitric acid solution, sodium or calcium chlorides for instance, are suitable sources.

The desmutting technique of the present invention is particularly desirable for use on surfaces that are not flat, or are not readily accessible for mechanical scrubbing. Thus an expensive sand-blasting operation is eliminated in the preparation of AN 355 jet engine blades for diffusion aluminizing and top coating by the process described in U.S. Pat. No. 3,948,689 and U.S. patent application Ser. No. 953,762 filed Oct. 23, 1978. (U.S. Pat. No. 4,241,147 granted Dec. 23, 1980). Such blades are very effectively given the following sequence of treatments.

#### EXAMPLE 5

The blades are subjected to steps (a), (b) and (c) of Example 4, followed by ultrasonic treatment of about 50,000 Hertz in tap water for one minute. They are then dipped in  $\frac{1}{2}\%$  by weight aqueous uninhibited hydrochloric acid, followed by the flash coating of step (f) in Example 4, but with only 30 seconds of cathodic action at 40 amperes per square foot. This is then followed by another rinse in tap water and a strip in 15% by weight

aqueous nitric acid containing 0.15% sodium chloride, another tap water rinse, a repeat of the foregoing ultrasonic treatment and another nickel flash coating. This flash coating is applied for two minutes at 40 amperes per square foot using the same nickel plating bath. The resulting flash-coated blade is rinsed in tap water, permitted to dry and packed in the aluminum diffusion coating pack of Example 1 in Ser. No. 953,762, and subjected to the diffusion coating there described. After the aluminizing the blades are removed from the pack, washed with tap water, and given the top coating of Example II of U.S. Pat. No. 3,948,689.

The resulting blade has a very smooth surface and a long life in a jet engine compressor.

The nitric acid strip solution should not be kept in contact with the ferrous surface for more than a few seconds after the flash is removed. While nitric acid tends to passivate ferrous surfaces, particularly when this acid is in a high concentration, the passivating action cannot be depended upon to persist very long when the metal is being manipulated.

Obviously many modifications and variations of the present invention are possible in the light of the above teachings. It is therefore to be understood that within the scope of the appended claims the invention may be practiced otherwise than as specifically described.

What is claimed:

1. In the stripping of aluminide diffusion cases from a superalloy surface by treatment with an aqueous solution of fluoride-containing nitric acid, the improvement according to which that treatment is followed by treatment with a bath consisting essentially of aqueous fluoride-free nitric acid and having a concentration between about 10 and about 30% by weight, for at least about 5 minutes.
2. The combination of claim 1 in which the aqueous essentially fluoride-free acid is at a temperature of about 80° to about 110° F.
3. The combination of claim 1 in which the stripping is effected by repeated alternating treatment with the fluoride-containing and fluoride-free nitric acids.

\* \* \* \* \*